

(No Model.)

J. E. WEST & C. O. WHIPPLE.

PROCESS OF MANUFACTURING ARTICLES OF PLASTIC MATERIAL.

No. 508,494.

Patented Nov. 14, 1893.

Fig. 1.



Fig. 2



Fig. 3.



Fig. 4.



Fig. 5



Fig. 6



Fig. 7.



Witnesses:

Sidney R. Hollingsworth  
William O'Connell

Inventors,  
Josiah E. West,  
Carlos O. Whipple,  
by their attorneys

Malcolm Davidson Night.

# UNITED STATES PATENT OFFICE.

JOSIAH E. WEST AND CARLOS O. WHIPPLE, OF ST. CLOUD, MINNESOTA,  
ASSIGNORS TO THE ST. CLOUD VULCANIZED FIBREWARE COMPANY,  
OF SAME PLACE.

## PROCESS OF MANUFACTURING ARTICLES OF PLASTIC MATERIAL.

SPECIFICATION forming part of Letters Patent No. 508,494, dated November 14, 1893.

Application filed May 19, 1893. Serial No. 474,826. (No specimens.)

*To all whom it may concern:*

Be it known that we, JOSIAH E. WEST and CARLOS O. WHIPPLE, citizens of the United States, residing at St. Cloud, in the county of Stearns and State of Minnesota, have invented certain new and useful Improvements in Processes of Manufacturing Articles of Plastic Material, of which the following is a specification.

10 The primary object of our invention is to manufacture buckets or pails of paper pulp, or similar fibrous material, having combined therewith a suitable binding agent; but, some parts or certain features of our improvements may also be employed in the manufacture of table tops, ornamental molding, electrical goods and various other similar articles.

15 We will show and describe our improvements as employed in the manufacture of paper pails, but we wish it understood that by suitably modifying the process and apparatus, other kinds of articles may be made.

20 Hollow ware articles have heretofore been extensively made from paper pulp by various processes, but generally by what is known as the wet process. There are very few instances in which hollow ware has been made in molds from granulated or powdered pulp, 25 but the latter way possesses many advantages, as the articles may be made hard and durable and capable of resisting the action of hot or cold water, acids and alkalies, by simply combining with the powdered pulp suitable substances.

25 So far as the invention claimed in the present case is concerned, the particular kind of fibrous material and binding agent employed is not important, but in order that our entire process may be fully understood, we would state that we preferably take ground wood pulp and mix it with chemical or sulphite pulp, preferably in a beating engine, but the mixture may be made in any kind of a 30 mixing machine; or, we may combine wood pulp or sulphite pulp with scraps of waste water-proof paper, as we find that by so doing, not only do we save material, which has heretofore been wasted, but we obtain an

improved result; or, we may take ground 50 wood pulp and mix it with say twenty-five per cent. of flax tow, previously cooked or steamed in lime water. In the beating engine, we treat the mixed pulp with a rosin sizing, which may be such as ordinarily employed in the 55 manufacture of paper, but we use more than the ordinary quantity. In connection with the rosin, we preferably employ lime after it has been slaked and impregnated with oil, tallow, or other grease, and to this mixture, 60 we add alum to set the sizing, and if it is desired to color the mixture, we add a suitable pigment. When thoroughly mixed, we transfer the pulp to a wet machine, to form it into sheets, or transfer it to vats to drain. After 65 being thoroughly dried, it is passed to a re-grinder, which granulates the pulp, great care being taken to prevent, as far as possible, the fiber from being powdered, and the resulting material is fluffy or like wood wool, and has 70 a gummy feeling. Preferably, while in the re-grinder, we add finely pulverized rosin as an additional binder. The material in this condition is now ready for the first or what we call the warm press. As before stated, 75 the selection of materials and the particular way of treating them does not form part of the invention herein claimed. They are claimed in our application for patent, Serial No. 450,227, filed October 28, 1892. 80

The steps of the process above described may be slightly varied. The mixing of the ground wood pulp and sulphite or chemical pulp or flax tow, or water-proof paper, can be effected after the ingredients have been dried 85 and re-ground, by placing them in a revolving mixing machine, at which time the rosin and treated lime may be added, and the pigment for coloring, if desired, may also be added at the same time. For the manufacture of some classes of articles, the rosin sizing may be omitted, but when such sizing is omitted, a larger quantity of pulverized rosin is added.

We will now state the manner of forming 90 articles, such as pails, according to our improved process.

We form in the warm press, above men-

tioned, the body or side of the pail, but instead of making it round or circular, we form the body flat, or substantially so, and also form at the edges suitable bevels or tongues 5 and grooves to make the seam or joint; or, we may form the edges in any suitable way so that they may match and when compressed will readily adhere to each other. This particular feature of our invention is claimed in 10 another application filed by us May 12, 1893, and serially numbered 473,944. In the warm press, the pulp is pressed into shape, not much pressure being required and that only for a short time. If it is desired to add strength- 15 ening strips or pieces of metal, or other like material, we first partially fill the warm press with pulp and then put the hoop, sheet or strip in position and then put in additional pulp and apply pressure. The bottom of the 20 pail may be formed in a similar press or warm die, or, as preferred, it may be formed by placing granulated material in the body blank and then compressing it into shape. After the body blank is formed into shape and allowed to cool, or immediately after it is taken 25 from the warm press, it may be treated with a coating of rosin oil, or if a large amount of pulverized rosin has been mixed with the pulp, then the blanks may be treated with lin- 30 seed oil. The amount of oil to be used may be varied according to the grade of pail required, and for cheap packing pails, this treatment will not be required at all. By this treatment, the oil permeates the blank and 35 assists in melting the rosin and binding the fibrous material together and making the pail water-proof. When water proofed paper or pulp has been used this treatment may be omitted. The pail blank thus formed and 40 treated, may then be taken to a former and bent into shape and allowed to cool. It is then transferred to a hot press or mold, and put in place and the pail bottom is applied, which may be done either by forming a circular or disk-shaped blank and uniting it 45 with the body, or, as we prefer, granulated material is placed in the body blank and is compressed and united with the blank in the hot press. When the body blank is thus 50 placed in the mold, and the granulated material is arranged in the blank, the plunger is lowered, and by putting on great pressure, say from two thousand to three thousand pounds to the square inch, the bottom is 55 formed and united to the body and the pail is completely formed. The binding material and oil are melted and caused to impregnate all portions of the body and bottom, and a substantially homogeneous or seamless article is produced. From the hot press, the pail 60 is taken to a cold press, which is slightly smaller than the hot press. It is there subjected to great pressure, and all blisters are removed from the surface of the pail, and it 65 is hardened and given a smooth finish. It is also in this press given its final form. The

pail is then taken from the cold press and baked in an oven for say twenty-four hours, beginning at a temperature of about 150° Fahrenheit, and gradually increasing to a temperature of about 250° Fahrenheit. The pail may then be finished by coating it with water-proof material, varnish, ebony finish, or other like material.

In the accompanying drawings, we have 75 shown diagrammatically the different steps of the process.

Figure 1 shows the warm, flat press where the body of the pail is formed. Fig. 2 is a view of the product of the warm, flat press. 80 Fig. 3 is a view of the former in which the body blank is bent into shape. Fig. 4 is a view of the product of the former. Fig. 5 is a view of the hot press. Fig. 6 is a view of the cold press, and Fig. 7, a view of the final 85 product.

A indicates the outer or female member of the warm press, and B, the plunger. As will be observed, they are both chambered and have entrance and exit pipes for the circulation of a heating agent. In order to form a beveled edge at each end of the blank, the bottom of the press is formed at a, with an inclined projection, and the plunger is formed at b, with a similar inclined rib or projection. 90 The material in a dry, granulated or fluffy condition is placed in the press, and pressure is applied which will cause the particles to cohere, and give to the mixture the desired form. If it is desired to embed a strip or 100 sheet of metal or other stiff material in the body of the blank, it may be done by first partially filling the mold A with granulated material, then placing a strip in position, then filling in more granulated material, and then 105 applying pressure. The pail blank, such as indicated in Fig. 2, is next taken to a former, such as shown in Fig. 3, where it is bent into the shape indicated in Fig. 4. It is then 110 taken to a hot press C, which comprises a plunger c, and an outer mold c', both of which are steam-heated. We then pour into the blank thus placed in the mold, a suitable quantity 115 of the combined fibrous material and binding agent, as indicated in Fig. 5, and then the plunger is made to descend, which first compresses the granulated material, flattens it to 120 form the bottom, and causes it to firmly unite with the body blank, which is in a comparatively loose condition, and readily permits the 125 granulated material forming the bottom to unite with it. Then, by applying heat and great pressure, the binding material is melted and caused to impregnate the pulpy or fibrous material, and the material is compressed and reduced to the desired thickness. The product of this press, however, is comparatively 130 loose and pliable, and while still warm and in this condition, it is transferred to the cold press, indicated in Fig. 6, where, instead of circulating a heating medium, we circulate a cooling agent and apply great pressure. This

press is slightly smaller than the hot press, in order that the material may be firmly compacted. In the cold press, all blisters are removed from the surface of the pail, and it is 5 hardened and given a smooth finish.

We attach great importance to the use of a cold press, as it enables us to remove the blisters and give the smooth finish, just referred to. From the cold press, the pail is taken to 10 an oven and baked a suitable length of time, say twenty-four hours, and may then be finished by coating it with water-proof material, varnish or the like.

Our complete process involves several steps, 15 and we have mentioned the use of numerous materials which may be employed. We desire to state, however, that so far as the broad features of our invention are concerned, the materials employed may be varied as may 20 also the steps of the process and the apparatus employed.

We claim as our invention—

1. The process herein described, for the manufacture of articles from fibrous material, 25 which consists in forming in a warm press from ground or powdered fibrous material, while dry and containing a binding agent, a blank for the article, then bending the blank into form, then subjecting the article to heat 30 and pressure to melt the binding material and thereby combine it with the fiber and

then subjecting the article to pressure and the action of a cooling agent.

2. The herein described process, which consists in forming a blank for an article of 35 fibrous material, and a binding agent, then treating the blank thus formed with oil or similar material, then cooling the article thus treated, and then subjecting it to heat and great pressure to melt and unite the binding 40 material to the fibrous material and to give form to the article.

3. The process herein described for the manufacture of hollow ware articles, which consists in forming from combined fibrous 45 material and a binding agent, while dry and in a fluffy or granulated condition, a blank for the body of the article, then partially filling the blank with the combined dried, granulated material and binding material, and then 50 by heat and pressure compressing and compacting this mixture to form the bottom of the article, and to firmly unite it to the body thereof.

In testimony whereof we have hereunto subscribed our names.

JOSIAH E. WEST.  
CARLOS O. WHIPPLE.

Witnesses:

L. T. TROUTMAN,  
JNO. BLATTNER.